

## UNITED STATES PATENT OFFICE

2,319,428

## RAYON MANUFACTURE

Arthur F. F. Mothwurf, Philadelphia, Pa., assignor, by mesne assignments, to Imperial Rayon Corporation, Gloucester, N. J., a corporation of Delaware

No Drawing. Application October 5, 1940,  
Serial No. 359,901

7 Claims. (Cl. 18—54)

This invention relates to the manufacture of artificial fibres or other regenerated cellulose products by the cuprammonium process and has as its particular object a novel method of regenerating cellulose from its cuprammonium solutions.

A further object of this invention is to effect this regeneration by fewer operations than were, heretofore, considered necessary.

Another important object of this invention is to lower the cost of the cuprammonium process.

Still other objects and advantages, inherent to the features and practice of our invention, will more fully appear in the following explanation:

When regenerating cellulose from cuprammonium cellulose solutions, for example in the production of artificial fibres, the treatment or treatments to be employed prior to final washing have to serve the two purposes of liberating their ammonia content and of converting copper content into a readily removable solution.

It is obvious that application of acids, by neutralizing ammonia and by dissolving copper, can take care of both purposes.

However, experience has shown that the action of acids is too rapid and that the ensuing thread is stiff and brittle and invariably uneven in structure and affinity for dyes.

Practice has, therefore, turned to other means of precipitation with a resulting preference for caustic soda in more or less diluted form.

Caustic, in contact with the spinning solution, expels ammonia from the soluble copper ammonia cellulose complex, and deposits most of the copper content of the latter as insoluble copper hydroxide within the coagulating thread which leaves the precipitating bath in a highly hydrated, semi-plastic state so that an acid treatment has to follow in order to free it from copper and to complete its deflation and setting.

Compared with the course of an acid precipitation, such proceeding adds at least one more operation and additional expenses for caustic and sulphuric acid which a one-stage coagulation would avoid.

The present invention provides a non-acid precipitating bath which offers all the benefits of a single treatment and eliminates at the same time the defects and inconveniences, which the application of free acid and subsequent neutralization would involve.

In principle, the composition of the new precipitating bath comprises two active components of which the first is able to absorb ammonia, while the second has to dissolve copper to a form in

which it is readily removed from the thread by subsequent washing, to which components neutral salts for physically influencing coagulation may be added.

As substances of the first description we select metallic salts which attract ammonia to enter therewith into compounds of higher stability than the copper-ammonia-cellulose complex. Such salts for instance are:

10 Copper salts, zinc salts, calcium chloride, sulphate of alumina, etc.

Components of the second description must be able to function as solvents for copper hydroxide in an alkaline solution. Ammonia salts, salts of oxycarbonic acids, like glycolates, tartrates, citrates, etc., or glycerine and its homologues, sugars and others can serve this purpose.

It is the substance of this invention, that no satisfactory results are obtained by combining 20 representatives of the two groups indiscriminately, but that the respective components have to be selected and proportioned with careful consideration of possible interreactions.

The following instance is meant to convey a clearer conception of this important point:

In practice, I prefer, for the sake of economy, to apply a combination of copper sulphate and ammonium sulphate.

Copper sulphate, acting as component of the 30 first description, absorbs ammonia, whereby the reaction goes successively through the following two stages:

I  $\text{SO}_4\text{Cu} + 2\text{NH}_3 = \text{Cu}(\text{OH})_2 + \text{SO}_4(\text{NH}_4)_2$   
II  $\text{Cu}(\text{OH})_2 + \text{SO}_4(\text{NH}_4)_2 + 2\text{NH}_3 = \text{SO}_4(\text{NH}_3)_4\text{Cu}$

35 which stages account for the fact, that in the presence of sufficient ammonia salt, copper sulphate will attract ammonia, forming without intermediate precipitate of copper hydroxide, soluble copper tetramine sulphate.

40 The reaction expressed by the second formula qualifies ammonium sulphate as the necessary solvent for copper hydroxide.

While it further implies that ammonium sulphate alone may act, in a chemical sense, as a one stage precipitant for cuprammonium cellulose solutions, such action is, in practice, predicated on the ratio of ammonia to copper hydroxide content of the spinning solution being approximately the same as stipulated by above equation or 0.35 to 1.

Such a condition is not applicable to our case: with all cuprammonium cellulose solutions that ratio is much higher (1.5—1.8 to 1). It introduces a large excess of ammonia against which

coagulating action of ammonium sulphate alone cannot materially develop beyond the purely physical effect of a salt solution.

To direct it definitely along the desired chemical line the presence of copper sulphate has been found expedient and effective. It engages the excess of ammonia and, thereby, leaves ammonium sulphate free to exercise its function as a solvent for copper hydroxide.

It can be seen that the amount of copper sulphate must be just sufficient to convert the prevailing surplus of ammonia into copper tetramine sulphate, in other words—and this is one of the special features of this invention—a constant chemical relation has to be maintained between the copper sulphate content of the precipitating liquid and the ammonia content of the spinning solution, otherwise coagulation will either slacken or basic copper hydroxide will precipitate.

To guard against the former possibility, I prefer to employ a small excess of copper sulphate and to prevent its precipitation by adding a corresponding amount of glycerine or corn syrup which addition has the further advantage of assisting in the removal of copper from the thread in the subsequent washing.

It will be further seen, that there is a minimum amount of sulphate of ammonia required as solvent, but that there is no limitation to any reasonable increase above that minimum amount; in fact, the margin left for the percentage of this component or for any neutral salt in its stead represents one of the various means of modifying coagulation. As the rate of diffusion rises with increasing temperature, another means of modification consists in the temperature at which the precipitating liquor is applied. Also other suitable additions such e. g. as favor or prevent deflation may be made.

The problem of reconditioning the withdrawn precipitating liquor for repeated use, which is of great consequence from an economical point of view, offers no difficulty; during the course of the reaction the entire ammonia and copper content of the spinning solution has been converted into copper tetramine sulphate.

The latter is subject to the following reactions:



II



Accordingly, sulphuric acid is added until all the copper is precipitated. Simultaneously, the entire ammonia has been transformed into ammonium sulphate slightly increasing the concentration of the liquid in this salt over the original percentage. To make proper adjustment a portion of the liquor, equivalent to said increase, is definitely withdrawn and treated for recovery of ammonia. For the balance enough copper hydroxide or basic copper sulphate is dissolved in sulphuric and enough water is added to restore original concentration of copper sulphate as well as the original volume.

Theoretically, the total amount of sulphuric acid needed should correspond to the ammonia content of the spinning solution—in practice, this amount is less due to loss of ammonia through adhesion to the thread, through evaporation and other causes—and may be further

lowered by forcing evaporation before adding the acid.

Economies effected by this method as compared with the favorite two stage caustic precipitation are substantial. Of the chemicals used in the two stage process there are saved the total of caustic, that part of the sulphuric which is required for its neutralization and the use of any additional chemicals for copper recovery.

10 In addition, the one stage method creates conditions very favorable for reclaiming ammonia.

Though a combination of copper sulphate and ammonia sulphate for precipitation involves a maximum of economy, and is therefore the most interesting phase of this invention, its principle can be extended to other combinations.

15 In giving instances of the manner in which this invention is carried out in practice, I relate them all to a spinning solution containing:

|                  | Percent |
|------------------|---------|
| Cellulose (100%) | 4       |
| Ammonia (100%)   | 3.6     |
| Copper hydroxide | 2.4     |

25 to a spinning speed of 64 meters (71 yards) per minute and to 150 denier yarn.

*Example #1*

The precipitating bath is made up as follows:

30 For each 1,000 cc.:

|                        | Grams  |
|------------------------|--------|
| Sulphate of ammonia    | 150    |
| Copper sulphate (100%) | 1.7288 |
| Glycerine              | .25    |

35 It circulates at ordinary temperature at a rate of 500 cc. per jet and per minute.

Of the 3.6% ammonia contained in the spinning solution, 2.76% represents what I have previously termed as excess ammonia.

40 The amount of copper sulphate is originally calculated to absorb this excess as copper tetramine sulphate. In the further course of precipitation the current requirements are established by tests and held at the point where additional copper sulphate creates cloudiness by precipitating copper hydroxide. Glycerine is added to provide for possible fluctuations of the copper sulphate content of the precipitating liquor.

50 During coagulation all available ammonia and copper hydroxide (except that held in solution by the glycerine) is converted into copper tetramine sulphate.

55 Under proper consideration of the losses of liquid, through adhesion to the thread and of the changes in volume, various methods may be employed for conditioning the withdrawing precipitating liquor for repeated use.

I prefer to proceed in the following manner: about one-eighth of the withdrawn precipitating liquor is by-passed. To the balance, which is recirculated, enough sulphuric acid is continuously added to precipitate all of the copper as basic compounds. The rate of flow necessary for this purpose is likewise controlled by tests. Taking into account the losses through adhesion, and by-passing, in the above example I found it to be around 1.30 grams of sulphuric acid, 60° Bé, per minute and litre.

60 After the copper precipitate is removed by filtration or otherwise, enough copper sulphate solution and water is added to restore the precipitating bath to its original volume and content of copper sulphate per litre.

Due to the precipitate being in the form of basic copper compounds of varying composition, I recommend the removal of all of the copper from the withdrawn precipitating bath and the utilization of fresh copper sulphate solution of known percentage in its restoration. This gives more accurate results than could be obtained by adding first an amount of sulphuric acid sufficient to precipitate all of the copper and then adding more acid to dissolve that portion of the precipitated copper needed for recirculation.

The by-passed portion is freed of the copper by acid, is neutralized with lime and is subjected to distillation for the recovery of ammonia.

The wash waters are treated for copper recovery only.

*Example #2*

The precipitating bath is made up as follows:

|                          | Grams | 20 |
|--------------------------|-------|----|
| Chloride of ammonia      | 150   |    |
| Chloride of calcium      | 2.4   |    |
| Glycerine; per 1,000 cc. | .25   |    |

It circulates at a temperature of 40-45° C. (104°-113° F.) and at a rate of 500 cc. per minute per jet.

The reactions which take place are similar to those of the preceding example; copper is dissolved to copper tetramine salt while ammonia combines with calcium chloride, so that reconditioning of the withdrawn liquor can be effected by muriatic acid.

It is, however, more advantageous in the case of recovery to precipitate the copper as copper sulphide, preferably with calcium sulphide, and to force evaporation of ammonia so that the amount of muriatic acid which is finally required for binding free ammonia is kept as low as possible. Incidentally, the portion of the withdrawn liquor which has to be by-passed is correspondingly reduced.

Precipitation of copper tetramine sulphate by acid is not the only way of reconditioning the withdrawn precipitating liquor. There are other possibilities as, for instance, removal of the excess or total copper content as copper sulphide, basic copper carbonate, etc. or evaporation of ammonia may be forced to effect precipitation of copper and to lower consumption of sulphuric acid or any one of these various methods may be used in conjunction with others.

There are and will be yet other modifications of my process at my hands and at the hands of others. Each and all of the modifications which conform to its generic spirit are intended to be protected to me through this patent application at large, irrespective of the circumstantial terminology of the claims appended.

What is claimed is:

1. The process of regenerating cellulose from its cuprammonium solutions in a single stage which consists in spinning the cuprammonium solution in an alkaline precipitating bath, which bath comprises, besides water as a solvent, two chemically active components, of which one is a copper sulphate for attracting and absorbing ammonia and the other of which is ammonium sulphate to dissolve copper hydroxide in an alkaline solution.

2. A process according to claim 1 in which the

concentration of the copper sulphate is during the spinning maintained at a constant chemical ratio to the ammonia concentration of the spinning solution, said ratio being such that substantially the whole of the ammonia content not otherwise consumed or lost during the reaction will be absorbed by said copper sulphate.

3. Process according to claim 1, in which the copper sulphate is introduced slightly in excess of that quantity substantially sufficient to bind that part of the available ammonia originating from the spinning solution that is not otherwise consumed during the reaction, said excess resulting in a precipitate, said ammonium sulphate being introduced to keep in solution said precipitate produced by the excess of said first component.

4. Process according to claim 1 in which the temperature of the precipitating bath is kept between 15° and 60° C.

5. Process of regenerating cellulose from a cuprammonium solution in a single stage which consists in spinning a cuprammonium solution in a precipitating bath comprising, besides water as a solvent, two chemically active components of which the first component is copper sulphate and the second component is ammonium sulphate, and the copper sulphate is not consequentially more than the amount necessary to absorb as copper tetramine sulphate that part of the ammonia content of the spinning solution which is not consumed in dissolution of the copper hydroxide of the spinning solution by the ammonium sulphate lost.

35 6. Process of regenerating cellulose from its cuprammonium solution which comprises the step of precipitating and decoppering in a single stage by the use of a spinning bath substantially the entire body of which is during the spinning continuously in a non-acid condition, which process comprises the further step of withdrawing at least part of the precipitating liquor containing copper sulphate and water and the withdrawn used precipitating liquor is reconditioned 40 for re-circulation, said process comprising the addition of sufficient sulphuric acid to precipitate all its copper content, the process comprising the further step of withdrawing for ammonia recovery a portion of the liquor that contains the total gain in ammonium salt due to the use of the bath, and the process comprising the step of restoring the remainder of the liquor to the composition and volume which the original precipitating bath possessed before its use, by the addition of copper sulphate and water.

7. Process of regenerating cellulose from its cuprammonium solution in which precipitation and decoppering are carried out in a single stage by means of one spinning bath, which bath contains copper sulphate and water, the process comprising the step of withdrawing precipitating liquor and reconditioning it for re-use by forcing precipitation of copper hydroxide and evaporation of ammonia to the extent of the gain in copper and ammonia from the immediately preceding use, removing the precipitated copper hydroxide, and restoring the liquor to its original composition and volume by the addition of copper sulphate and water as necessary.

ARTHUR F. F. MOTHWURF.